

May 21, 1957

C. N. CONE ET AL.

2,792,616

## METHOD FOR SHRINKING FABRIC

Filed May 25, 1955

2 Sheets-Sheet 1



**INVENTORS**  
CLARENCE N. CONE &  
LEE A. HUGHES  
BY *Campbell, Brumbaugh*

their ATTORNEYS

May 21, 1957

C. N. CONE ET AL

2,792,616

METHOD FOR SHRINKING FABRIC

Filed May 25, 1955

2 Sheets-Sheet 2



FIG. 1B.



INVENTORS  
CLARENCE N. CONE &  
LEE A. HUGHES  
BY *Campbell, Bunnough,  
Lee & Stevens*

Their ATTORNEYS.

# United States Patent Office

2,792,616

Patented May 21, 1957

1

2,792,616

## METHOD FOR SHRINKING FABRIC

Clarence N. Cone, Greensboro, and Lee A. Hughes, Brown Summit, N. C., assignors, by mesne assignments, to Levi Strauss and Company, San Francisco, Calif., a corporation of California

Application May 25, 1955, Serial No. 511,043

2 Claims. (Cl. 26—18.5)

This invention relates to fabric shrinking apparatus and methods and more particularly to fabric shrinking apparatus and methods whereby the shrunken fabric retains to a very large degree its initial ability to withstand wear.

Shrinking methods and apparatus are widely used for treating fabrics before they are made up into garments or the like to minimize further shrinkage of the fabric in the hands of the consumer. The presently most generally used so-called preshrinking processes are harsh in their treatment of the fabrics in that they involve various warpwise mechanical compressive methods and sometimes weftwise stretching methods often accompanied by elevated temperatures and pressures at critical points sufficient to materially reduce the resilience and strength of the fabric and impair the life of the fibers themselves. The overall effect has been a fabric of reduced wearing properties. This invention is particularly applicable to fabrics such as heavy denims of the order of 11 oz. to the yard which are primarily used in garments in which heavy, rugged wear is of utmost importance. Previously such fabrics have been considered difficult to preshrink satisfactorily but may now be easily treated to obtain desired properties.

In accordance with the present invention, there are provided apparatus and methods by means of which fabric can be shrunk prior to its use in apparel or the like with no damage to the fabric or its ability to withstand hard use. This shrinkage further is of a type which has improved cutting and garment making characteristics and minimized subsequent area changes of an undesirable nature. This desirable result has been achieved by subjecting the fabric to simulated natural relaxing forces which tend to bring it into equilibrium conditions. The cloth after weaving is passed through a series of operations including wettings and subsequent dryings with material flexing but without at any time placing the fabric under radical stress, particularly tension or compression, either warpwise or weftwise. It is also to be noted that this invention permits a high throughput of fabric, however, without the utilization of any special equipment both of which factors are essential to a successful and competitive operation in this field.

A representative embodiment of the invention from which the above and other features thereof can be readily understood by those skilled in the art is described below having reference to the accompanying drawings in which:

Figure 1A is a diagrammatic view in side elevation of the first stages of an apparatus for carrying out the invention; and

Figure 1B is a diagrammatic view in side elevation of the concluding stages of the apparatus illustrated by Figure 1A.

Referring now to the drawings, placing Figures 1A and 1B end to end, the complete apparatus is shown carrying out the process of the present invention. The fabric F is illustrated in dot-dash lines entering the ap-

2

paratus at the left hand end of Figure 1A and leaving at the right hand end of the complementary Figure 1B. The fabric as produced on the looms usually is cut into lengths of about 60 yards and delivered to the finishing department where it is classified as to color or style, combined in lengths of about 1000 yards by sewing the goods end to end, sheared, brushed and inspected. These are conventional steps and, of course, may be varied considerably without materially modifying the subsequent steps comprising the invention.

The fabric F then passes downwardly into a wetting out box 10 containing known desired wetting, softening, sewing and other treating agents.

A suitable and effective wetting agent is desired at this point inasmuch as it is an important factor in the process that the fabric be rapidly and effectively wet at intervals in order to relax the warp and filler yarns and assist them in combination with other elements of the invention in reaching equilibrium conditions. The first treatment must be effective in penetrating rapidly any prior additive remaining on the fabric from the weaving and prior operations. The use of wetting agents in textile processing is well known and any of the known penetrants for that purpose may be used. For example, 20 sulphonated compounds, sold under the trade name "Triton X" have been found effective. Softening agents or lubricants such as sulphonated oils, sulphonated tallow may be used. Sulphonated tallow, sold under the trade name "Estol T Sulfonated" has been found effective. Sulphonated mineral oils such as those sold under the trade name "Twitchell" oils are known wetting, softening agents for cotton textiles.

The geometry of the wetting out box and the amount of the wetting and treating agent contained therein are related to the speed of travel of the fabric to afford an exposure in the bath of about 0.6 second, the temperature of the agent being about 120° F. In a representative process and apparatus a fabric speed of 25 yards per minute was used. The fabric can be held beneath the liquid level of the treating agent in the wetting out box 10 by guide means 11 and 12, preferably in the form of freely rotating rollers. The latter guide means 12 can also serve as one element of squeezing means formed by the companion rollers 12 and 13 having resilient surfaces and 30 carried by a suitable supporting frame work 14 having suitable adjusting means for regulating a compression on the rollers 12 and 13. The rollers 12 and 13 are so disposed above the wetting out box 10 that the residual liquid returns to the box. Passing upwardly from the squeeze 35 rolls the wetted fabric is carried by conveyer means 15 which can take the form of a canvas duct belt conveyer, one pulley 16 of which can be mounted on the frame 14 and another pulley 17 of which can comprise the first 40 can of a first drying cylinder stack indicated generally by the numeral 18.

The stack 18 includes, in addition to the can 17, a plurality of successively laterally offset cans 19, 20, 21, 22, 23, 24, 25 and 26, all supported for rotation about 45 horizontal axes, and all driven in rotation in successively opposite directions as indicated by the direction of arrows in each, through a suitable adjustable drive means (not shown). The fabric F is passed from can to can moving back and forth and upwardly to the top of the stack 18, with the speeds of rotation being adjusted to impose minimum warpwise strain on the fabric. The travel of the fabric over the first can 17 is slightly greater than the subsequent surface speed over the cans of the conveyer 15 which in effect gives can 17 a greater diameter than the subsequent cans. This small degree of

overfeed from can 17 precludes tensioning of the fabric in the stack 18.

From the top of the stack 18 the fabric F is passed without tension through a succession of driven drying stacks passing downwardly and upwardly in sequence through each to a final drying stack 27 corresponding generally to the stack 18 and arranged to carry the fabric downwardly with minimum strain imposed thereon to an out feed guide in the form of a freely turning roller 28. Between successive drying stacks the fabric is maintained in a relaxed condition by appropriate adjustment of the drive means which are individually adjustable for the several stacks. The fabric at all points between stacks and when passing to subsequent equipment, it is to be noted, is in a relatively loose, sagging condition and is supported by rollers or endless belts.

The cans of the several stacks are heated, in accordance with preferred practice, by steam to a temperature in the range of 160° to 180° F. Somewhat higher or lower temperatures may be used with the understanding (a) that the heat must be sufficiently high at this point, as well as at later heating zones, to influence the tendency of the fabric to move toward a shrunk equilibrium condition in combination with the other steps disclosed and (b) must be sufficiently low to avoid adversely affecting the fibers of the fabric resulting in loss of life, resiliency and wear resistant qualities.

The fabric initially charged at the wetting box 10 may normally have a shrinkage of about 10% warpwise for example. Coming off of the last stack warpwise contraction or shrinkage will have been reduced about 50% and may be of the order of 5 or 6%. The fabric relatively free from stress or tension in its travel to this point in a wet condition initially and after being flexed many times, begins to assume a preshrunk condition resulting from tendency of the warp and weft threads within the fabric to reach an equilibrium under these conditions.

Passing from the last stack of drying cylinders the fabric is in a relatively stiff boardlike condition and passes to a flexing and driving frame assembly indicated generally by the numeral 29 with the fabric passing under and over relatively closely spaced and vertically offset rollers 30, 31 and 32 to a pair of complementary feed rolls 33 and 34, the latter pair being driven from a variable speed transmission 35 to a belt coupling 36 in order to minimize tension in the fabric. Passing in an S configuration through the driven feed rolls 33 and 34, the fabric is passed over a pair of vertically spaced guide rolls 37 and 38 to effect a vertical downrun adjacent water spray means 39 which can take the form of a water spray nozzle 40 supported on a shelf 41.

Passing from the lowermost guide roll the water sprayed fabric passes upwardly and around the major part of the circumference of a drying cylinder 42 driven from the variable speed transmission through belt means 43. A second drying cylinder 44 is journaled for rotation about a horizontal axis below the cylinder 42 and is driven therefrom by belt means 45, with a guide roller 46 engaging the fabric between the cylinders 42 and 44 to control the wrap of the fabric thereabout. Emerging from the cylinder 44 the fabric path is controlled by guide rollers 47, 48 and 49 to pass to a supporting or carrier roll assembly indicated generally by the numeral 50. The temperature of the drying rollers 42 and 44, which are preferably heated by a suitable medium such as steam for example, is maintained in the range between roughly 160° and 180° F. and the speed of driving of the drying cylinders 42 and 44 is so adjusted through the variable speed transmission 35 with respect to the speed of driving of the feed rolls 33 and 34 to preclude insofar as possible tensioning of the fabric warpwise, with suitable compensations being made as

necessary to accommodate the contractions occasioned by the fabric shrinkage.

Passing from the carrier assembly 50 the fabric is passed over a battery of scrimp bars 51, which again flex the fabric, from which it is conveyed to a conventional Palmer 52 for completion of the drying operation and to impose a final finish. The Palmer 52 includes a large rotatable heated drum 53 around the major portion of the circumference of which the fabric is passed. The heated drum 53 is engaged over a major portion of its circumference by an endless belt 54, which between its points of engagement with the drum 53 is conveyed over a series of guide rollers 55, 56, 57, 58, 59, 60 and 61, the latter being disposed at the point of introduction of the blanket 54 to the circumference of the drum to define the nip into which the fabric is conventionally introduced. The Palmer 52 is driven from a suitably controlled driving source (not shown) to achieve a desired throughput which, in accordance with the present invention, is related to the speed of the drying cylinders 42 and 44, the feed rolls 33 and 34, the several stacks of drying cylinders, of which 18 and 27 are representative, and the wetting out box and squeeze roll assembly 10, 12 and 13 so as to impose no warp tension upon the fabric. The Palmer is heated to a temperature of between about 280° and 300° F.

Passing from the scrimp bars 51 the fabric to be introduced into the Palmer is passed over a guide roll 62 which is so disposed relative to the nip defined by the guide roller 61 and the drum 53 that the fabric is introduced to the Palmer at a point at which the belt 54 is in a relatively unflexed condition, i. e., the surface of the belt 54 which engages the fabric at the nip has assumed a curvature no greater than that of the drum 53, which is relatively large. In this fashion, the fabric passes into and through the Palmer without the application of warpwise bunching or compressing forces applied thereto. The finished fabric is conveyed from the Palmer 52 to a suitable storage means (not shown) by guide rollers 63, 64 and 65.

Additional wetting zones may be provided as the fabric moves through the processing apparatus, if desired. Also additional related heating and flexing elements may be provided as desired along the route of the fabric if it is noted that the characteristics of a given fabric or garment product from such fabric would be better served by such modification to the disclosed process. The presently disclosed process and equipment has been found to be effective with heavy denims suitable for the best work garment wear, particularly those requiring fabrics with the greatest life, resiliency, abrasive resistance such as to saddle wear.

The final fabric ready to ship to the consumer has been found to have a warpwise shrinkage of the order of 1% and a weftwise shrinkage of about 3% or less with no additional processing steps applied. The shrinkage test used is the standard (A. S. T. M.) for the industry. In the tables below examples of shrinkage and abrasive tests have been set forth as typical but not limiting. The abrasive test was also standard in the industry (A. S. T. M.) using a rotary platform double head abraser of the type made by the Taber Instrument Company.

|    | Shrinking Tests—<br>Heavy Denims |                                 |
|----|----------------------------------|---------------------------------|
|    | Cloth from<br>Loom,<br>percent   | Finished<br>Cloth, per-<br>cent |
| 65 |                                  |                                 |
| 70 | Example I:<br>Warpwise.....      | 10.2                            |
|    | Fillingwise.....                 | 6.16                            |
|    |                                  | .86                             |
|    | Example II:<br>Warpwise.....     | 11.23                           |
|    | Fillingwise.....                 | 6.93                            |
|    |                                  | 3.83                            |
|    |                                  | 1.96                            |
|    |                                  | 3.53                            |

It will be noted that the present invention gives an ef-

fective and notable preshrunk condition to the cloth. This is accomplished with a rapid throughput, with an assembly of conventional equipment, and without harsh treatment of the fabric. The fabric is not overshrunk warpwise as is often the case with conventional compression shrinking methods, resulting in subsequent stretching which is undesirable from the garment cutters' standpoint. The filling or weftwise shrinkage of about 3% is not considered undesirable from the garment cutters' viewpoint because of the manner or direction in which the filling is positioned in the garment.

| Abrasive Test—Heavy Denims (Additives Removed by Washing) |                           |                                                                                   |
|-----------------------------------------------------------|---------------------------|-----------------------------------------------------------------------------------|
|                                                           | Finished Cloth, rotations | Cloth Preshrunk by Conventional Method Using Compression and Hot Irons, rotations |
| Example A.....                                            | 683                       | 634                                                                               |
| Example B.....                                            | 751                       | 626                                                                               |

These abrasive tests illustrate by way of typical examples the material improvement in wearing qualities of the products of the herein disclosed invention.

We claim:

1. A process for rapidly and continuously imparting equilibrium conditions to a woven fabric consisting in treating the fabric with a wetting and penetrating agent to soften and relax the fibres of said fabric, subsequently

5 continuously flexing said fabric in a substantially untensioned condition while subjected to temperatures of not greater than about 180° F., subsequently continuously rewetting said fabric, and continuously flexing and heating said fabric in a substantially untensioned condition at temperatures not greater than 180° F.

10 2. A process for continuously and rapidly producing a resilient woven fabric with maximum strength and wear-resistant properties having the warp and filler threads in substantially equilibrium condition, said process being free from harsh temperatures and mechanical compressive action in the plane of the fabric and being performed entirely in a condition substantially free from mechanically imposed tensions on said fabric, comprising 15 continuously passing said fabric through a wetting zone whereby the threads of said fabric are softened and relaxed, subsequently continuously passing said fabric through a flexing zone in a substantially untensioned condition while subjecting said fabric to temperatures of about 160° to 180° F., rewetting said fabric and again 20 continuously flexing said fabric in a substantially untensioned condition at temperatures of about 160° to 180° F., and finally flexing and subjecting said fabric to a pressing action with heat whereby a fabric of good finish and 25 superior wearing and preshrunk qualities is produced.

References Cited in the file of this patent

UNITED STATES PATENTS

|              |                        |               |
|--------------|------------------------|---------------|
| 30 2,327,712 | Huey et al. .....      | Aug. 24, 1943 |
| 2,338,983    | Thackston et al. ..... | Jan. 11, 1944 |
| 2,584,753    | Spooner .....          | Feb. 12, 1952 |